

## [54] CLAY PREPARATION

[75] Inventors: Claud L. Stratton; James F. Kane,  
both of Benton, Ark.[73] Assignee: Reynolds Metals Company,  
Richmond, Va.

[21] Appl. No.: 61,300

[22] Filed: Jul. 27, 1979

[51] Int. Cl.<sup>3</sup> ..... C22B 1/24

[52] U.S. Cl. ..... 75/3; 75/5

[58] Field of Search ..... 75/3, 4, 5

## [56] References Cited

## U.S. PATENT DOCUMENTS

|           |        |                        |           |
|-----------|--------|------------------------|-----------|
| 3,192,290 | 6/1965 | Polon .....            | 23/313 X  |
| 3,240,562 | 3/1966 | Brown et al. ....      | 423/132 X |
| 3,864,118 | 2/1975 | Schumacher et al. .... | 75/3      |

Primary Examiner—G. Ozaki

Attorney, Agent, or Firm—Glenn, Lyne, Girard &amp; McDonald

## [57] ABSTRACT

There is described a novel process for pelletizing clay containing aluminous ore comprising the steps of:

- crushing the clay to within an appropriate size range;
- blending the crushed clay with water to achieve a closely defined moisture content;
- pelletizing the clay in a suitable apparatus to provide clay pellets of predetermined size;
- rolling the pellets for a period of time sufficient to round the edges, corners, etc. and to produce a relatively hard, abrasive resistant surface; and
- drying and calcining the pellets at a temperature within the range of from about 1100° to about 1500° F.

4 Claims, 2 Drawing Figures





FIG. 1

SERIAL NO. 061300  
GROUP ART UNIT III

FIG. 2

## CLAY PREPARATION

## FIELD OF THE INVENTION

The present invention relates to a method for preparing various ore containing clays for processing and extraction of the ore values and more particularly to a method for pelletizing aluminous ore containing clays for acid or other extraction of the aluminous values therefrom.

## BACKGROUND OF THE INVENTION

With the decline in the availability of high aluminum content ores throughout the world and a desire to make use of lower assay domestic clays numerous processes have been suggested and developed for the extraction of aluminum values from such "low" assay clays. Of particular interest in recent years have been the so-called "acid" extraction techniques. According to these techniques, the clay is treated with an acid, usually nitric, hydrochloric or sulfuric, to extract the aluminum values which are subsequently purified and refined according to a variety of conventional or novel methods.

In any such extraction process the first step is to place the clay in a condition such that it can be treated with an appropriate acid to yield the aluminum values while leaving the clay behind. Numerous clay preparation methods have been described and are generally well known to those skilled in this art.

With the evolution of the fluidized or expanded bed and the development of extraction techniques using this operation, the clay preparation step becomes even more crucial to the development of successful commercial clay extraction techniques.

Most alumina digestion operations described in the literature comprise the co-current digestion, over a substantial period of time, of powdered or coarse-ground calcined kaolin at atmospheric or superatmospheric pressure, followed by a large number of stages of counter-current decantation washing of the solids separated from the product liquor. Even when using coarsely-ground calcined clay from which fines have been separated before leaching, the requirements for maintaining the co-currently digesting slurry in a mixed condition, and for obtaining good mixing between the settled solids and wash liquors in the countercurrent decantation washing stages, are impossible to fulfill without the generation of excessive quantities of very fine silicious slimes of around 10 micron and down particles. The slimes settle very slowly, and only to relatively dilute slurries. Large amounts of water, that must be subsequently evaporated, and many washing stages are required to obtain washed slimes which still may contain excessive quantities of acids. However, production by the process herein described of size-tailored pellets, with all the initially-induced edges, corners and protruding areas rounded off toward the spherical shape, permits practice of counter-current digestion and washing methods that avoid the aforesaid washing difficulties and which also can provide a product liquor containing dissolved alumina in excess of stoichiometric requirements. Such pelletizing when using nitric acid leaching permits use of an essentially zero-energy-requirement process for the removal of iron and silica values to levels sufficiently low that the final specifications with regard to these elements can be obtained in a crystallization process.

Many methods, mostly expensive, are well known in the art for preparing pellets of kaolin clay which can then be calcined to provide feed for digestion. We have used in the early stages of our investigations cylindrical extrusions produced by forcing properly-moistened clay through sized holes in a die, and round balls produced by agglomeration of dried, ground clay with water on a pelletizing disk.

## BRIEF DESCRIPTION OF THE DRAWINGS

FIGS. 1 and 2 are graphs showing particle size distribution of product pellets formed under a variety of screen sizes and moisture contents according to the practice of the instant invention.

SUMMARY OF THE INVENTION

The present invention provides a novel clay preparation technique which provides pelletized clay admirably suited for extraction of aluminum values by counter-current acid extraction.

In the clay preparation process of the present invention as mined clay is crushed to within an appropriate size range, blended with water to a closely defined moisture content, and passed through a hammer-mill or other suitable equipment of appropriate design to provide clay pellets of a specified screen size. The resulting sized pellets are then rolled, substantially without agglomeration, for a period of time sufficient to round the edges, corners, etc. and produce a relatively hard, abrasion resistant surface, i.e. the pellets are "surface hardened" by rolling. The rolled pellets are then dried by appropriate means and calcined at a temperature within the range of from about 1100° to about 1500° F., preferably in a fluidized bed heated by in-bed combustion of a suitable fuel.

## DETAILED DESCRIPTION

According to the present invention, as-mined clay crushed to a suitable maximum size by known means is blended with what additional water may be required, in, for instance, a mix muller, to obtain an intimate mixture of moisture and clay of a defined moisture content and is then passed through a suitable apparatus, for example, a hammer-mill comprising rotating knives on a vertical shaft surrounded by a 360° screen of specified aperture preferably between about 2 and about 8 mm, to produce a relatively narrow size range of damp particles. A preferred size range for the pellets is between about 1 and about 8 mm. Such particles or pellets are subsequently rolled in a drum, while taking due care to prevent agglomeration, for a relatively short period to press all jagged edges and the like into a relatively firm surface which tends toward a spherical shape and which is relatively resistant to abrasion, i.e. the pellets are "surface hardened". At the proper moisture content the particle size range of the product is controlled by the selection of the size of openings in the 360° product discharge screen of the hammermill or other suitable apparatus. The free moisture content, i.e., other than water of hydration, is critical to the operation and must be held within somewhat narrow limits which vary somewhat with the composition of the kaolin material. Thus a sand-free kaolin material, but with variable iron oxide impurity content, requires a moisture content between about 19 and 21% but produces a more desirable size distribution at levels between 19 and 20%. At moisture levels of about 22% this material will blind the screens and pile up on the hammers and shaft requiring

the mill to be shut down and cleaned out. At 18% moisture the product is essentially fine material unsuitable for the intended usage. Silica sand, which is frequently present in the kaolin bed, decreases the water requirement but does not prevent processing to suitable pellets at the proper moisture content. Thus a material which assays 21% silica and on a dry solids basis causes screen blinding at moisture contents of 18½% and above, but is processable at 18% moisture. The optimum moisture content is judged to be between about 17.5 and 18%.

On the other hand the introduction of calcined fine material, such as might be recovered from the off gases of a fluid bed calciner, increases the moisture content requirement, presumably because some water is absorbed into the pores of the calcined material. One such material, comprising 80 parts (dry weight basis) clay and 20 parts recycled calcined material, produced satisfactory pellets at a moisture level of 22%. Pellets formed by the tornado mill-screen combination described hereinabove are rolled to flatten out angular projections, corners and the like to minimize undesirable attrition in the fluid bed calciner and during digestion and handling of the fired pellets. A simple but efficient means for accomplishing this is a device, known to the art as a rolling drum, which consists essentially of a large diameter, long pipe or tube which may, if desired, contain one or more lifter means. As the drum or pipe is rotated pellets are fed at a feed end and pass slowly down the slightly inclined tube for a period of time which can be defined by the length of the tube and the inclination of the tube to the horizontal. In the passage, the pellets impinge upon each other and roll along the sides of the tube with the concurrent impartation of energy to the surfaces of the pellets whereby protruding areas are pushed inwardly to the pellet body, the surfaces are smoothed and rounded, and the pellet is gradually massaged toward a spherical shape. It is also known to generate pellets by agglomeration in such devices, however in the instant case the desired pellet masses have already been generated so that it is necessary to minimize further agglomeration to prevent growth of the particles into undesirably large sizes. The rolling drum could of course be used to produce pellets in the first place, however, we have found that the maximum pellet size and the pellet size distribution is exceedingly difficult to control in a manner to produce, per pass, an economical proportion of pellets within the size ranges desired for the digestion operation.

The pellet should be subjected to the rolling action of the drum for periods upwards of at least 5 minutes but we have found that by 30 minutes rolling the pellets are sufficiently compacted that further improvement is slow. As the pellets are rounded and surface-hardened by the peening action of the bed of pellets and of the metal shell, water is forced to the surface of the pellet, increasing their stickiness and thereby facilitating agglomeration of the particles into undesirably large masses.

The time required in the rolling drum to develop an undesirable sticky surface varies somewhat inversely with the moisture content of the materials entering the rolling drum. Thus pellets made with 21% moisture will begin to develop undesirable agglomeration tendencies within about 5 or 10 minutes.

Pellets produced at 19% moisture have been rolled successfully for 15 to 20 minutes while pellets which are dried to 18½% moisture before introduction into the rolling drum have been rolled for 30 minutes or more

(up to 60 minutes). By the use of a standardized attrition test, which comprised digesting a small amount of the calcined clay pellets with nitric acid in a cylindrical bomb while rotating the bomb at a constant rate and at the conclusion of the digestion period measuring the concentration of attrited solids suspended in the liquor decanted from the bomb, it was found that low attrition rates were favored by longer rolling times at moisture contents of 18½% or higher, with the lowest attrition rates being obtained for pellets predried to 18½% moisture and rolled for 30 minutes. We have found however that the same benefits can be obtained without the need of the separate drying step if the pellets are rolled in the presence of a draft of relatively dry air, whereby at least a portion of the aforesaid generated surface moisture is removed as it is formed under conditions which do not bring about substantial drying of the interior of the pellet. Little or no heating of the air is required because in a continuous flow process the pellets enter the rolling drum already warm, i.e., above ambient temperature, from the conversion into heat of the energy imparted to the material during mulling and milling.

Calcination of the pellets for the aforesaid standardized attrition tests were carried out at 1350° F. in the laboratory furnace with the production of low attrition rates and high solubility of the contained alumina. Similar tests using product calcined at higher temperatures gave lower attrition rates while preserving the same solubility of the contained alumina at calcination temperatures up to 1550° F. It is of course well known in the art that 1550° F. is about the maximum calcination temperature that can be employed without reducing the solubility of the contained alumina. Since, as is well known, the alumina solubility is excellent for calcination temperatures between about 1100° and 1550° F., the practitioner has available a wide temperature range for calcination. However, the range is restricted considerably by the choice of fuel and the choice of the calcination equipment. Thus when using methane, temperatures must exceed about 1400° F. for proper combustion. Only a little lower temperatures can be used with fuel oil or with coal. Rotary calciners are somewhat difficult to control sufficiently to operate at temperatures, for instance, high enough to utilize natural gas while at the same time preventing over-burning of at least a portion of the material. This difficulty is surmounted with use of a fluid bed calcining means which, as is well known in the art, can be controlled easily to within a range of 15° to 30° F. of a specified temperature so that even a 1500° F. bed temperature may be used without danger of creating hot spots in the bed.

Thus by the aforesaid relatively inexpensive method of preparing substantially rounded pellets within a size range eminently satisfactory for use in fluid beds, and in themselves relatively resistant to attrition, we are able to calcine the said pellets within the temperature range of about 1500° to 1550° F. without danger of overburning any of the material, and at the same time obtain the benefits of the lower attrition rates so provided.

#### EXAMPLE 1

The following practices, for which particle size distribution data are presented in FIGS. 1 and 2, indicate generally the effect of screen size and moisture content on product size distribution. Materials for these tests were milled in a laboratory-size mix-muller of standard design. The blended damp material then was passed through a 10½" diameter tornado mill, Model 44-0, man-

ufactured by the Stokes Machine Company, using various screen sizes as indicated, and the resulting pellets were rolled in a 55 gallon drum in which two  $1\frac{1}{2}$ " wide by  $\frac{1}{4}$  thick steel plates had been welded lengthwise to the side of the drum to serve as lifters.

Referring to FIG. 1, the size distributions of the product from the use of each of the 5 different size screens on the tornado mill are shown in curves A, B, C, D and E. Curve D, which was made with a 3 mesh screen with square openings of about 6.7 mm formed by 1.87 mm wire and with 20% moisture content in the clay, shows a particularly desirable size distribution. This was the average size distribution while processing of material containing 550 pounds of dry solids through the tornado mill and then rolling for 15 minutes. This material contained only a minor amount of +6 mm material, and only 5% of minus 1 mm material from which a satisfactory portion could be removed easily by passing over a 16 or 18 mesh screen. Curves A, B, C and E were obtained with 0.8 mm, 3.35 mm, 4.75 mm and 12.7 mm square-opening screens respectively, with about 21% moisture in the clay feed.

A Product D which was ground at about the optimum moisture content of 20% gives a substantially straight line distribution whereas products A, B, and C ground at about 21% moisture, departed from the straight line relation in the direction of the formation of excessive amounts of very fine particles. It is thought that Product E, which was also ground at 21% moisture, indicates a beneficial effect of reducing the rotation rate of the knives in the tornado mill from a normal 3500 rpm to 2200 rpm. The increased production of fines with damper material is indicated also in curves F and G of FIG. 2 in which curve F was ground at 21% moisture through a half inch U.S. Sieve series screen and Curve G, which exhibits a lower proportion of fines, was ground through the same screen at 19% moisture. Curve G is substantially parallel to Curve D. Products H and K indicate the influence of some diluents, Product H comprising 20% (dry weight basis) of calcined and ground clay and ground at 22% moisture, and Product K comprising a mixture of sandy clay and nonsandy clay blended to provide 21% sand (dry basis) and ground at 18% moisture. From the slopes of the curves compared to Curves D and G it is thought that both of these products contained slightly more water than the optimum.

It is of course preferred to control moisture content to a specific value as determined by any number of well known methods of determination including drying the material at 105° C. In addition, however, we have found that several observations and/or tests readily performed by the operator can be used as guides for adjusting the moisture content as, for instance, the quantity of sand in the clay being fed might change from time to time. As

5 aforesaid, the slopes of the product pellet size distribution presented in FIGS. 1 and 2, which are readily determinable by well known methods of screening, are useful for indicating when the moisture content is about right or it might be lowered slightly to improve product size distribution. We have also noticed that, when the moisture content is about right, small balls of a quarter inch or so diameter tend to form in the muller during the mulling operation. This action can serve as a quick visual check on the adequacy of the moisture content. As the moisture content increases beyond desirable levels, the lumps become larger and appear wetter and eventually will become quite pasty. Conversely, as the moisture content decreases below the desirable level, the balls become smaller, tending toward grains, and mulled material compressed in the hand into lumps will tend to fall apart when the hand pressure is released.

10 15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9925 9930 9935 9940 9945 9950 9955 9960 9965 9970 9975 9980 9985 9990 9995 10000 10005 10010 10015 10020 10025 10030 10035 10040 10045 10050 10055 10060 10065 10070 10075 10080 10085 10090 10095 10100 10105 10110 10115 10120 10125 10130 10135 10140 10145 10150 10155 10160 10165 10170 10175 10180 10185 10190 10195 10200 10205 10210 10215 10220 10225 10230 10235 10240 10245 10250 10255 10260 10265 10270 10275 10280 10285 10290 10295 10300 10305 10310 10315 10320 10325 10330 10335 10340 10345 10350 10355 10360 10365 10370 10375 10380 10385 10390 10395 10400 10

TABLE-continued

| RUN NO.                                     | EXAMPLE 2 |      |      |      |      |      |      |      |      |      |      |      | 31   | 25   | 26   | 19   | 21   | 22   |
|---------------------------------------------|-----------|------|------|------|------|------|------|------|------|------|------|------|------|------|------|------|------|------|
|                                             | 17        | 11   | 12   | 13   | 14   | 16   | 24   | 18   | 30   | 1350 | 1350 | 1550 |      |      |      |      |      |      |
| Firing Temp. - °F.                          | 1350      | 1350 | 1350 | 1350 | 1350 | 1350 | 1350 | 1350 | 1350 | 1350 | 1350 | 1550 | 1350 | 1350 | 1550 | 1600 | 1500 | 1550 |
| Attrited Solids                             |           |      |      |      |      |      |      |      |      |      |      |      |      |      |      |      |      |      |
| % in liq.                                   | 1.34      | 0.54 | 1.19 | 1.01 | 2.24 | 1.55 | 1.84 | 1.28 | 2.54 |      |      |      | 2.04 | 1.21 | 1.16 | 0.79 | 0.99 | 0.18 |
| % of pellet charge                          | 4.8       | 1.9  | 4.3  | 3.6  | 8.1  | 5.6  | 6.6  | 4.6  | 9.1  |      |      |      | 7.3  | 4.4  | 4.2  | 2.8  | 3.6  | 0.6  |
| Particle Preparation                        |           |      |      |      |      |      |      |      |      |      |      |      |      |      |      |      |      |      |
| % Moisture                                  | 21        | 21   | 21.5 | 20   | 18.1 | 22   | 18   | 22   | —    |      |      |      | 20.0 | 20.0 | 20.0 | 21   | 21   | 21   |
| Screen Aperture, mm                         | 12.7      | 12.7 | 12.7 | 12.7 | 12.7 | 12.7 | 12.7 | 12.7 | —    |      |      |      | 6.7  | 6.7  | 6.7  | 12.7 | 12.7 | 12.7 |
| % Fe <sub>2</sub> O <sub>3</sub> - Raw Clay | 4.7       |      |      |      |      |      |      |      | 13.5 |      |      |      | 10.5 |      |      |      |      |      |

The bomb was charged with 150 grams of the 4.8 on 1 mm size range pellets and 520 grams of a 40% nitric acid-in-water solution, closed, placed in the harness within the already-hot-oven, and rotated at 13 rpm for 240 minutes. The bomb was then removed from the oven and cooled and the residual pellets were separated from the slurry by pouring the slurry through a screen with about 1 mm square apertures. Solids passing through the screen with the liquor were separated from the liquor, washed with water, dried and weighed.

This attrition test is believed to provide more strenuous attriting conditions than would be obtained during fluid-bed calcination of the pellets or in counter-current extraction of the pellets by passage of digestion liquor through fixed, expanded, or partially-or-totally-fluidized beds of pellets.

### EXAMPLE 3

A 4-inch diameter by 2½ inch deep bed of about 4.8+1 mm undried and unfired pellets, comprising 19.68% free moisture, and produced as in test 26, of Example 2, was subjected to a series of compression forces up to 7 psi acting through a 4-inch diameter vertical piston in accordance with appropriate weights gently placed upon the top of the piston. A thirty-minute settling period after imposition of each pressure increment was allowed before measuring the bed compression. The loose bed compacted about 24% but the pellets did not agglomerate and showed very little change in surface appearance or overall shape. A gentle

rolling action in the palm of the hand was sufficient to separate the individual pellets from each other.

From the foregoing, it is apparent that the clay granulation technique described herein provides particulate clay optimally suited to extraction in fluid or expanded bed techniques.

What is claimed is:

1. A process for pelletizing clay containing aluminous ore comprising the steps of:
  - a. crushing the clay to within an appropriate size range;
  - b. blending the crushed clay with water to achieve a moisture content of between about 17.5 and about 22 percent by weight water;
  - c. pelletizing the clay in a suitable apparatus to provide clay pellets of predetermined size;
  - d. surface hardening the pellets; and
  - e. drying and calcining the pellets at a temperature within the range of from about 1100° to about 1500° F.
2. The method of claim 1 wherein the pelletizing is performed using a hammermill comprising rotating knives on a vertical shaft surrounded by a 360° screen having an aperture size of between 2 and about 8 mm.
3. The method of claim 1 wherein said surface hardening is accomplished by rolling the pellets in a rolling drum.
4. The process of claim 3 wherein the rolling is performed for a period of between about 5 and about 60 minutes.

\* \* \* \* \*

45

50

55

60

65